

1

3,282,847

### HYDRAULIC FLUIDS

Karl Schneider, Leverkusen, and Hans-Werner Kauczor, Cologne, Germany, assignors to Farbenfabriken Bayer Aktiengesellschaft, Leverkusen, Germany, a corporation of Germany  
No Drawing. Filed July 28, 1965, Ser. No. 475,571  
5 Claims. (Cl. 252—78)

The present invention relates to hydraulic fluids; more particularly it concerns hydraulic fluids based on aryl- or alkylaryl esters of phosphoric acid, which possess an active amount of the amides produced from aliphatic or araliphatic amines and halides of partially esterified phosphoric acid.

This application is a continuation-in-part application of our co-pending application Serial No. 182,977, filed March 21, 1962, and now abandoned.

Suitable amides are for example obtainable by reacting, preferably in a molecular proportion of 1:2-4, phosphoric acid diphenyl ester monochloride, phosphoric acid octyl phenyl ester monochloride, phosphoric acid dicresyl ester monochloride, and phosphoric acid dicresyl ester monobromide with aliphatic or araliphatic amines, such as e.g. 2-ethylhexylamine, n-octylamine, di-n-butyl amine, dodecylamine, oleylamine, stearylamine, benzylamine, and  $\omega$ -phenyldodecylamine, with heating if required, in an inert organic solvent, in which the simultaneously formed hydrochlorides of the amines are insoluble, for instance in ligroin, removing the salts and evaporating the solvent.

The content of the amides in the hydraulic fluids amounts in general to 0.1 to 15 percent by weight, preferably 0.5 to 5 percent by weight.

If desired, chlorinated hydrocarbons, such as chlorinated paraffin, chlorinated diphenyl, and chlorinated terphenyl, or polyethers, such as those from tetrahydrofuran and 1,2-oxide compounds, can be added to the hydraulic fluids in order to improve the non-inflammability or the viscosity temperature characteristics. The hydraulic fluids can also contain further additives, usual for hydraulic fluids, e.g. stabilizers, thickeners, antifoaming agents, anticorrosives and de-emulsifiers.

The hydraulic fluids of the present invention possess outstanding lubricant properties. On account of the content of the amides herein before defined only very small frictional forces are set up even in the range of boundary lubrication. The parts given in the following table are by weight.

TABLE

|                                                                                                                                                                                  | Friction in kg. <sup>1</sup> |
|----------------------------------------------------------------------------------------------------------------------------------------------------------------------------------|------------------------------|
| (I) Tricresyl phosphate                                                                                                                                                          | 260                          |
| Mixture of 98 parts of tricresyl phosphate and 2 parts of the amide produced from phosphoric acid diphenyl ester monochloride and dodecylamine                                   | 150                          |
| (II) Mixture of 50 parts of tricresyl phosphate and 50 parts of tetrachlorodiphenyl                                                                                              | 240                          |
| Mixture of 49 parts of tricresyl phosphate, 49 parts of tetrachlorodiphenyl, and 2 parts of the amide produced from phosphoric acid diphenyl ester monochloride and dodecylamine | 170                          |

<sup>1</sup> Measured at 1000 kg. applied pressure on the Almen-Wieland machine. Cf. Zerbe, Mineralöle und verwandte Produkte (1952), 907-908.

2

Friction in kg.

(III) Diphenyl xylene phosphate ----- 300

    Mixture of 97 parts of diphenyl xylene phosphate and 3 parts of a polyether obtained by copolymerization of tetrahydrofuran, ethylene oxide and 1,2-propylene oxide and possessing an average molecular weight of 6000 ----- 260

    Mixture of 95 parts of diphenyl xylene phosphate, 3 parts of the above mentioned polyether and 2 parts of the amide produced from phosphoric acid diphenyl ester monochloride and dodecylamine ----- 155

The amide applied was produced from phosphoric acid diphenyl ester monochloride and dodecylamine in the following manner:

Within one hour 670 g. (3.6 mol) of dodecylamine were added dropwise to a solution of 472 g. (1.75 mol) of phosphoric acid diphenyl ester monochloride in 500 ccm. of ligroin while the reaction temperature was kept at 35-40° C. by cooling. Thereupon the reaction mixture was stirred at room temperature for a further three hours, then shaken three times with 2 normal sodium hydroxide solution and finally distilled in vacuo. After the solvent and the excess of dodecylamine were distilled off the amide produced distilled at 210-270° C./0.5 mm. Hg. The yield amounted to 823 g.

Similar favourable results are obtained if instead of the amide produced from phosphoric acid diphenyl ester monochloride and dodecylamine the other amides are applied which are obtainable in the same manner as herein before described from the amines and partially esterified phosphoric acid halides mentioned above.

We claim:

1. A fluid composition consisting essentially of (A) a hydraulic fluid consisting of a member selected from the group consisting of aryl ester and an alkylaryl ester of phosphoric acid and (B) about 1-15% by weight of an amide additive obtained by reacting (a) a component selected from the group consisting of 2-ethyl hexylamine, n-octylamine, di-n-butyl amine, dodecylamine, oleyl amine, stearyl amine, benzylamine, and  $\omega$ -phenyldodecylamine with (b) a component selected from the group consisting of phosphoric acid diphenyl ester monochloride, phosphoric acid octyl phenyl ester monochloride, phosphoric acid dicresyl ester monochloride, and phosphoric acid dicresyl ester monobromide, the molar proportion of (b) to (a) being about 1:2-4.
2. The composition of claim 1 containing at least one additional additive in a flame-retarding amount, the additive being a member selected from the group consisting of tetrachlorodiphenyl, and a copolymerization product of tetrahydrofuran, ethylene oxide and 1,2-propylene oxide, said copolymerization product possessing an average molecular weight of 6000.
3. A fluid composition containing 98 parts of tricresyl phosphate and 2 parts of the amide produced by reacting phosphoric acid diphenyl ester monochloride with dodecylamine.
4. A fluid composition containing 49 parts of tricresyl phosphate, 49 parts tetrachlorodiphenyl, and 2 parts of the amide produced by reacting phosphoric acid diphenyl ester monochloride with dodecylamine.

5. A fluid composition containing 95 parts of diphenyl xylene phosphate; 3 parts of a polyether having an average molecular weight of 6000 produced by copolymerization of (a) tetrahydrofuran (b) ethylene oxide and 1,2-propylene oxide; and 2 parts of the amide produced by reacting phosphoric acid diphenyl ester monochloride with dodecylamine.

2,994,638 8/1961 Malz et al. \_\_\_\_ 260—461.306 X  
2,995,596 8/1961 Debo \_\_\_\_\_ 252—77 X  
3,056,745 10/1962 Morschel et al. \_\_\_\_\_ 252—78

5 LEON D. ROSDOL, *Primary Examiner.*

JULIUS GREENWALD, ALBERT T. MEYERS,

*Examiners.*

References Cited by the Examiner

UNITED STATES PATENTS

2,933,449 4/1960 Moreton \_\_\_\_\_ 252—78 X

10 R. D. LOVERING, *Assistant Examiner.*